

## UNITED STATES PATENT OFFICE

2,676,099

PROCESS OF COATING FIBERS WITH GAS  
AGITATIONJohn Y. L. Kao, Chicago, Ill., assignor to F. D.  
Farnam Co., Chicago, Ill., a corporation of  
IllinoisNo Drawing. Application September 25, 1948,  
Serial No. 51,294

5 Claims. (Cl. 92—21)

1

The present invention relates to a process for coating animal, mineral or vegetable fibers, and particularly to a process for coating such fibers while in the pulp state with any material which can be emulsified.

There are in commercial use today many methods of coating fibrous material with a coating either before or after the fibrous material has been formed into sheets. Of these processes, the present invention is concerned only with those wherein the pulp is treated prior to being formed into sheets.

The conventional means and methods for treating pulp with latices or emulsions of resinous material and the like have not, until this invention, been changed or improved in any major particular for about a quarter of a century.

The conventional process of so treating pulped fibers is known as the beater process or the beater saturation process. This prior art process requires the use of the conventional pulp beater which is loaded with sufficient pulp to raise the concentration of the pulp to as high as 5% or 6% because this prior process at best is slow and if a lower concentration were used it would raise the cost of the process to an uneconomically high value. However, with the pulp at this high concentration the fibers tend to entangle and intertwine forming clumps of fibers. The viscosity of the pulp slurry is high and as the pulp slurry is passed through the beater, there is little or no dispersion of the fibers in the water or pulp liquor—only the slow movement of a stream or mass of pulp fibers except when the pulp passes through the beater blades at which time its movement is greatly accelerated.

This prior art process was primarily developed for coating pulp fibers with rubber. However, when the rubber latex and coagulant were added to the pulp in the beater, the result indicated that the rubber coated the outside of the clumps of fibers with only a small percentage of rubber. It is obvious that with the rubber coating primarily the outer surfaces of the clumps that all of the fibers in the pulp will not have a uniform coating of rubber.

Because the pulp slurry has a high viscosity neither the latex nor the coagulant will be properly dispersed and local high concentrations of latex or coagulant will occur causing local and spotty coagulation of the latex to form clumps of rubber and rubber threads. This is particularly true of latices which are not properly or completely stabilized. These rubber formations and clumps of pulp plug the screen during the

2

paper making and will also damage the pump and flow conduits.

Another reason for the presence of clumps of rubber in the pulp slurry is in the use of the beater to circulate the pulp during the prior art process. As the pulp is circulated the clumps of pulp coated with rubber come into direct contact with the rapidly rotating blades. Since the rubber is not firmly attached to the pulp fibers, it may be—and frequently is—stripped off and small particles of coagulated rubber will be free in the pulp slurry.

It is obvious that the prior art process produces a pulp that is very difficult to work on the paper or sheet forming machine. The finished product lacks uniformity due to the loss of rubber in the formation of clumps of rubber and due to the uneven distribution of the rubber on the pulp fibers. This lack of uniformity is demonstrated by corresponding deficiencies in the physical characteristics of the finished sheet product.

As a result of these difficulties it is not commercially feasible, using the prior art processes, to manufacture a finished product having a uniformly deposited material content of greater than about 20% of the weight of the product.

The principal object of the present invention is to provide a novel process of coating fibers in the pulp stage with an emulsifiable material which overcomes the foregoing difficulties of the prior art processes.

Another object is to provide a novel process for treating fibers with an emulsifiable substance wherein the finished product may contain up to 55% or more of the deposited coated substance by weight.

Another object is to provide a novel process for treating fibers in the pulp stage with an emulsifiable substance wherein the fibers are so agitated and dispersed that each individual fiber is uniformly and evenly coated with the substance.

Another object is to provide a novel process for coating fibers in the pulp stage with an emulsifiable substance wherein the treated pulp is substantially free from rubber or resinous lumps, clumps of fibers or uncoated fibers.

Another object is to provide a novel process of treating fibers with a substance such as natural and synthetic rubber, thermoplastic and thermosetting resins, waxes and oils, provided that the substance can be emulsified and can be added to the pulp in the form of an emulsion.

Another object is to provide a novel process of coating fibers in the pulp stage wherein the pulp is agitated in such a manner as to reduce the

coating time to under that required by the prior art processes.

Another object is to provide a novel process of coating fibers in the pulp stage so that the finished product has highly uniform physical properties.

Another object is to provide a novel process of coating fibers in the pulp stage wherein the pulp concentration in the slurry is substantially lower than that used in the prior art processes.

Another object is to provide a novel process of coating fibers in the pulp stage wherein the means for agitating and dispersing the pulp fibers includes no mechanical devices such as beaters or pumps or agitators and wherein the agitation and dispersion are more complete than in the prior art processes.

Other objects and advantages will become apparent from the following description. There are no drawings.

The present invention contemplates processing animal, mineral and vegetable fibers and no distinction among these fibers will be made in this specification. Examples of fibers that may be processed are wool and leather fibers (animal), asbestos (mineral), and wood and other cellulosic fibers (vegetable). In the specific examples set forth hereinafter the pulp is comprised of wood fibers.

Inasmuch as this invention in no way affects the preparation of the pulp, it may be prepared according to any one of the various processes now in commercial use. At the end of the beater operation the pulp should be diluted to a concentration of 2% or less and preferably 1% or under. This low concentration is preferred because at this concentration there is little or no tendency to form clots or clumps of fibers as is the case with pulp slurry in its normal concentration prior to dilution. Furthermore, the viscosity of the pulp slurry approaches that of water which makes its agitation easier thus increasing the dispersion of the fibers to increase the surface area of the fibers available for coating.

The pulp slurry is transferred to an agitation tank which preferably is a cylindrical vessel wherein the side walls curve into the bottom, which may be concave, so as to remove any sharp corners or crevices which could create dead spots or local eddy currents which would upset or disturb the regular and even—though very turbulent—agitation of the pulp slurry. Agitation is not carried out by any mechanical device but by means of air or a gas which is substantially water insoluble and non-reactive with water, pulp or added substances and which is introduced through strategically located jets or outlets in the bottom of the tank. The location of the jets or outlets forms no part of the present invention, but it is essential that they be located so that the entire mass of the pulp will be continuously agitated and so that the fibers will be given a turbulent movement and completely dispersed to inhibit the formation of clumps of fibers. Both the mass and turbulent movements are very rapid so as to facilitate the dispersion of the fibers and the emulsion or latex. As the air bubbles to the surface of the liquid in the tank it expands also to aid in the dispersion of the pulp fibers.

The gas which is used is preferably air, nitrogen, or a similar gas which is substantially insoluble in water and has no chemical effect upon the pulp, emulsion or latex. However, there may be occasions when a gas may be chosen for its

chemical activity—such as chlorine—so as to obtain a particular result. It is preferred that air be used because it may be compressed and filtered in the mill without the necessity of allocating storage space for tanks as would be the case were nitrogen to be used. It is essential that the gas be free from dust, dirt and other impurities. The gas is admitted to the tank at such a rate as to obtain a complete and substantially instantaneous dispersion of the emulsion or latex which is added to the agitated pulp at a controlled rate.

After the pulp has been transferred to the agitation tank, it is agitated as described and the agitation is continued until the end of the process. Next the coagulant is added to the ebullient slurry and the agitation is continued for five to ten minutes or such a time as is necessary for the coagulant to be thoroughly mixed with or dispersed in the pulp and for it to be adsorbed onto the surfaces of the pulp fibers before the emulsion is added. The coagulant is in the form of polyvalent cations, such as the water soluble salts of calcium, aluminum and thorium. It is not practical to use a monovalent cation since too large a volume of coagulant is necessary to provide the necessary electrical charge. The coagulant is added in such quantities and concentrations as required for the different emulsions and latexes.

While all the coagulant can be added at one time, it is preferable that the coagulant be added in two portions, the first portion containing less than the calculated total amount of coagulant required, and the second portion containing the remainder of the coagulant substantially diluted. It is preferred that the first portion of coagulant be between 50% and 90% of the amount required depending upon the nature and character of the pulp fibers and the emulsion; less than 50% does not seem to be satisfactory.

It is known that most of the pulp fibers are negatively charged or can easily be rendered negatively charged. Fibers of this charge have a great tendency to adsorb the polyvalent cations and thus to form on their surfaces a layer of positive charges, which will attract the negatively charged resinous or rubber particles. Due to the character of the coagulant—its water solubility—it will be adsorbed evenly by the fibers. The power of the coagulant to destabilize the emulsified material is dependent upon the total power of the electrical charge. Therefore, for the equivalent concentration of coagulant, thorium, a tetravalent cation, will have more coagulating power than aluminum, a trivalent cation, and aluminum will be more powerful than calcium, a divalent cation. Consequently, care must be used so as not to add an excess of coagulant before the addition of the emulsion, otherwise local coagulation will occur before the resin or rubber or the like is deposited upon the fibers. It is for this reason that it is preferred that less than all of the required coagulant be added to the pulp before the addition of the emulsion or latex.

The next step in the process is the addition of the emulsion or latex. It is added at such a rate that it will substantially immediately disperse into a pulp slurry. To accomplish this most effectively the emulsion or latex should be fed directly into the center of the agitation, either dropwise or in a small stream. The resinous or rubber particles will be attracted to the fibers

by their positive charge and will be evenly deposited thereon due to the evenness of the distribution of the charge. There will be no clumps of fibers because the gas agitation keeps the fibers well dispersed and moving constantly with both turbulent and mass movement. No lumps of resin or rubber will be formed because there is no excess of coagulant and because the particles are attracted to the fibers before they can be attracted to each other.

The emulsion or latex may or may not require the use of stabilizers, such as ionizable or non-ionizable soaps, and protective colloids, such as casein, glue and haemoglobin. The emulsion or latex preferably is diluted to a concentration of between 5% to 10% by weight of solids, although more dilute concentrations appear to be satisfactory.

As the addition of the emulsion continues the pulp liquor may become milky, and the viscosity of the pulp will increase due to the addition of the solids. It may be necessary to increase the rate of air flow so that the speed and character of the agitation will be properly maintained.

After all of the emulsion or latex has been added to the pulp slurry, the second addition of coagulant is made to exhaust the latex or emulsion. Since the pulp liquor contains particles of resin or rubber or the like the second addition must be made carefully to prevent local coagulation. The concentration of the coagulant for the second addition is, therefore, very much more dilute than the first, and it is added slowly while the pulp is continuously agitated as before. After the second addition of coagulant the pulp liquor should be free from any latex or emulsion, and the end point in this step is actually determined by the water or liquor becoming clear.

Pulp fibers treated according to this process will have a coating of resinous or rubber or the like particles throughout their entire length. The density and thickness of the coating will depend upon the amount of solid material added in the form of emulsion or latex. However, there will always be uniformity regardless of the density or thickness.

In order that the versatility of the process may be understood a few examples of pulp treated according to the hereinabove described process will be set out hereinbelow:

#### Example No. 1

| Material                                         | Concen-<br>tration<br>(Percent) | Dry<br>Weight<br>(Grams) | Wet<br>Weight<br>(Grams) |
|--------------------------------------------------|---------------------------------|--------------------------|--------------------------|
| Pulp.....                                        | 1                               | 20                       | 2,000                    |
| Water.....                                       |                                 |                          | 5,000                    |
| Aluminum Sulphate.....                           | 1                               |                          | 150                      |
| Latex of Buna Synthetic Rubber,<br>Type III..... | 20                              | 24                       | 120                      |
| Aluminum Sulphate.....                           | 0.125                           |                          | 400                      |

The rubber latex was stabilized and diluted to about 2% to 3% solids. After the first addition of aluminum sulphate the pulp was agitated by air for ten minutes, as was done in each of the other examples herein described, and the complete process carried out as set forth above. The total synthetic rubber in the coated pulp was slightly more than 54½%.

In this, and subsequent examples, reference to Buna synthetic rubber type III is meant G. R. S. synthetic rubber type III.

#### 6 Example No. 2

| 5  | Material                                         | Concen-<br>tration<br>(Percent) | Dry<br>Weight<br>(Grams) | Wet<br>Weight<br>(Grams) |
|----|--------------------------------------------------|---------------------------------|--------------------------|--------------------------|
|    | Pulp.....                                        | 1                               | 20                       | 2,000                    |
|    | Water.....                                       |                                 |                          | 5,000                    |
|    | Aluminum Sulphate.....                           | 1                               |                          | 150                      |
| 10 | Latex of Buna Synthetic Rubber,<br>Type III..... | 20                              | 20                       | 100                      |
|    | Curing Agent (dispersion).....                   | 50                              | 2                        | 4                        |
|    | Aluminum Sulphate.....                           | 0.125                           |                          | 200                      |

The process was carried out in exactly the same fashion as Example No. 1 except that the dispersion of curing agent was added after the latex and before the second addition of aluminum sulphate. In this process curing agents such as antioxidants, activators, sulphur and accelerators in the form of dispersions may be added—but if so should be added before the second addition of coagulant. In Example No. 2 the solids are 52.4% of the total.

#### 25 Example No. 3

| 30 | Material                                         | Concen-<br>tration<br>(Percent) | Dry<br>Weight<br>(Grams) | Wet<br>Weight<br>(Grams) |
|----|--------------------------------------------------|---------------------------------|--------------------------|--------------------------|
|    | Pulp.....                                        | 1                               | 20                       | 2,000                    |
|    | Water.....                                       |                                 |                          | 5,000                    |
|    | Aluminum Sulphate.....                           | 1                               |                          | 150                      |
| 35 | Latex of Buna Synthetic Rubber,<br>Type III..... | 20                              | 15                       | 75                       |
|    | Curing agent (dispersion).....                   | 50                              | 1.5                      | 3                        |
|    | P-33 (dispersion).....                           | 50                              | 5                        | 10                       |
|    | Aluminum Sulphate.....                           | 0.125                           |                          | 200                      |

In this example, a pigment, carbon black (P-33), was added to the pulp in a dispersion immediately after the addition of the latex and curing agent but before the second addition of aluminum sulphate. Such pigments are added for a variety of reasons such as to impart color or to increase the tensile strength of the sheet material made from the pulp. If a pigment is to be incorporated it may be mixed with the emulsion or latex or added separately in a dispersion. If added separately it must be added before the second addition of coagulant. The percentage of added solids in Example No. 3 is approximately 51.8% of the total weight.

#### 55 Example No. 4

| 60 | Material                                            | Concen-<br>tration<br>(Percent) | Dry<br>Weight<br>(Grams) | Wet<br>Weight<br>(Grams) |
|----|-----------------------------------------------------|---------------------------------|--------------------------|--------------------------|
|    | Pulp.....                                           | 1                               | 20                       | 2,000                    |
|    | Water.....                                          |                                 |                          | 5,000                    |
|    | Aluminum Sulphate.....                              | 1                               |                          | 150                      |
| 65 | Latex of Neoprene Synthetic<br>Rubber, No. 571..... | 20                              | 15                       | 75                       |
|    | Curing agent (dispersion).....                      | 50                              | 4.5                      | 9                        |
|    | P-33 (dispersion).....                              | 50                              | 2.75                     | 5.5                      |
|    | Acrawax C. (dispersion).....                        | 33½                             | 1.33                     | 4.0                      |
|    | Aluminum Sulphate.....                              | 0.125                           |                          | 200                      |

The amount of added solids is 51.6% of the total weight. P-33 is carbon black. "Acrawax C." is the trade name for a wax sold by Glycol Products Co. of New York. It is added in dispersion in the same manner as a pigment and increases the water resistance of the finished product.

## 7 Example No. 5

| Material                                    | Concen-<br>tration<br>(Percent) | Dry<br>Weight<br>(Grams) | Wet<br>Weight<br>(Grams) |
|---------------------------------------------|---------------------------------|--------------------------|--------------------------|
| Pulp                                        | 1                               | 20                       | 2,000                    |
| Water                                       |                                 |                          | 5,000                    |
| Aluminum Sulphate                           | 1                               |                          | 150                      |
| Latex of Buna Synthetic Rubber,<br>Type III | 20                              | 13.25                    | 66.25                    |
| Curing agent (dispersion)                   | 50                              | 2                        | 10                       |
| Acrawax C. (dispersion)                     | 33 1/2                          | 0.67                     | 2                        |
| Para-formaldehyde (dispersion)              | 50                              | 0.25                     | 5                        |
| Aluminum Sulphate                           | 0.125                           |                          | 200                      |

The amount of added solids is 44.6%. The dispersion of para-formaldehyde was added after the addition of the latex and before the second addition of aluminum sulphate.

## Example No. 6

| Material                | Concen-<br>tration<br>(Percent) | Dry<br>Weight<br>(Grams) | Wet<br>Weight<br>(Grams) |
|-------------------------|---------------------------------|--------------------------|--------------------------|
| Pulp                    | 1                               | 20                       | 2,000                    |
| Water                   |                                 |                          | 5,000                    |
| Aluminum Sulphate       | 1                               |                          | 150                      |
| Latex of vinyl chloride | 20                              | 20                       | 100                      |
| Aluminum Sulphate       | 0.125                           |                          | 200                      |

The latex of vinyl chloride is that sold by B. F. Goodrich Co. under its trade-mark "Geon"; it is type PX-8. The latex was diluted to 2% to 3% solids. This is an example of an added thermoplastic type resin, which constituted 50% of the weight of the finished product.

## Example No. 7

| Material                | Concen-<br>tration<br>(Percent) | Dry<br>Weight<br>(Grams) | Wet<br>Weight<br>(Grams) |
|-------------------------|---------------------------------|--------------------------|--------------------------|
| Pulp                    | 1                               | 20                       | 2,000                    |
| Water                   |                                 |                          | 5,000                    |
| Aluminum Sulphate       | 1                               |                          | 150                      |
| Latex of Styrene, X-580 | 20                              | 20                       | 100                      |
| Aluminum Sulphate       | 0.125                           |                          | 400                      |

Styrene X-580 is a vinyl type, thermoplastic resin manufactured by Dow Chemical Co. The latex was diluted to 2% to 3% solids.

## Example No. 8

| Material                                 | Concen-<br>tration<br>(Percent) | Dry<br>Weight<br>(Grams) | Wet<br>Weight<br>(Grams) |
|------------------------------------------|---------------------------------|--------------------------|--------------------------|
| Pulp                                     | 1                               | 20                       | 2,000                    |
| Water                                    |                                 |                          | 5,000                    |
| Aluminum Sulphate                        | 1                               |                          | 150                      |
| Durez's Phenolic Resin Emulsion<br>14170 | 20                              | 20                       | 200                      |
| Aluminum Sulphate                        | 0.125                           |                          | 600                      |

The resin is of the phenol formaldehyde thermosetting resin and its emulsion is sold by Durez Plastics & Chemicals, Inc. under the No. 14170. It has a pH value of 5 and was diluted to 2% to 3% solids.

## Example No. 9

| Material                                    | Concen-<br>tration<br>(Percent) | Dry<br>Weight<br>(Grams) | Wet<br>Weight<br>(Grams) |
|---------------------------------------------|---------------------------------|--------------------------|--------------------------|
| Pulp                                        | 1                               | 20                       | 2,000                    |
| Water                                       |                                 |                          | 5,000                    |
| Aluminum Sulphate                           | 1                               |                          | 150                      |
| Latex of Buna Synthetic Rubber,<br>Type III | 20                              | 8.3                      | 41.5                     |
| Emulsion of Plasticizer "Cumar"             | 20                              | 2.8                      | 14.0                     |
| 25 Resin                                    | 50                              | 2                        | 4                        |
| Curing agent (dispersion)                   |                                 |                          |                          |
| Aluminum sulphate                           | 0.125                           |                          | 200                      |

7 The amount of added solids is 39.5% of the total weight. The latex of Buna rubber was stabilized and blended with the "Cumar" 25 resin emulsion and then diluted to 2% to 3% solids. 5 "Cumar" 25 resin is a petroleum product.

## 8 Example No. 10

| Material                                       | Concen-<br>tration<br>(Percent) | Dry<br>Weight<br>(Grams) | Wet<br>Weight<br>(Grams) |
|------------------------------------------------|---------------------------------|--------------------------|--------------------------|
| Pulp                                           | 1                               | 20                       | 2,000                    |
| Water                                          |                                 |                          | 5,000                    |
| Aluminum Sulphate                              | 1                               |                          | 150                      |
| Latex of Neoprene Synthetic<br>Rubber, No. 571 | 20                              | 8.3                      | 41.5                     |
| Ester type plasticizer emulsion                | 20                              | 2.8                      | 14.0                     |
| Curing agent (dispersion)                      | 50                              | 1.5                      | 3                        |
| Aluminum Sulphate                              | 0.125                           |                          | 200                      |

20 The ester type plasticizer is sold by Monsanto Chemical Co. under the designation B-16. It was diluted to 2% to 3% solids.

25 After the pulp has been treated according to the present invention to coat the individual fibers with a rubber, resinous or the like material, the pulp may be formed into sheets on a conventional machine operated in the conventional manner.

30 Some of the finished products made from the improved sheeting formed from pulp treated according to this invention include gaskets, sheet packing, high strength papers, water and oil resistant papers, backing for pressure sensitive adhesives, imitation leathers, electrical insulating boards and panels, and the like.

35 While preferred embodiment and examples of the invention have been described, it will be appreciated that numerous changes, variations and modifications may be made in the process without departing from the spirit and scope of the invention. What is claimed as new and desired to be secured by United States Letters Patent is:

40 1. In the process of preparing a coated fibrous material, the improvement which consists in providing an aqueous slurry containing not more than about 2% of fiber, subjecting the slurry continuously to rapid, turbulent mass agitation by bubbling upwardly therethrough a gas whereby the fibers are continuously dispersed by the expanding gas bubbling therethrough, and slowly adding to the ebullient slurry a coating material in the form of an emulsion whereby the dispersed fibers are uniformly coated with the coating material.

45 2. The process as set forth in claim 1 in which a coagulant is added to the slurry prior to the introduction into the slurry of the coating material, to thereby precondition the fibers for the reception and retention of the coating material, and a more dilute coagulant is added to the ebullient slurry after the coating of the fibers has commenced to thereby achieve substantially 100% retention of the coating material by the fibers.

50 3. The process as set forth in claim 1 in which the coating material is a rubber latex and in which the latex emulsion contains about 2 to 10% of solids.

55 4. The process of coating fibers with emulsifiable material which comprises providing a dilute aqueous slurry of the fibers with the fiber content of the slurry being not more than 2% by weight, subjecting the slurry continuously to rapid, turbulent mass agitation by bubbling upwardly therethrough a gas whereby the fibers are

continuously dispersed by the expanding gas bubbling therethrough, and slowly adding to the ebullient slurry in the form of an emulsion a coating material selected from a group comprising natural and synthetic rubber, thermoplastic and thermosetting resins, waxes and oils, and in which the emulsion contains from about 2 to 10% solid material, said coating material being effectively dispersed throughout the slurry by said ebullient gas agitation whereby the dispersed fibers are uniformly coated with the coating material.

5. The process as set forth in claim 4 in which a polyvalent coagulant is added to the slurry with from about 50 to 90% of the coagulant being added prior to the introduction into the slurry of the coating emulsion and the remainder is added to the slurry in more dilute form during the coating step to obtain substantially complete retention of the coating material by the fibers.

20

## References Cited in the file of this patent

## UNITED STATES PATENTS

| Number    | Name        | Date          |
|-----------|-------------|---------------|
| 981,098   | McCaskell   | Jan. 10, 1911 |
| 1,502,686 | Schidrowitz | July 29, 1924 |
| 1,607,519 | Ellis       | Nov. 16, 1926 |
| 1,673,047 | Hawley      | June 12, 1928 |

| Number       | Name           | Date           |
|--------------|----------------|----------------|
| 1,971,852    | Goebels        | Aug. 28, 1934  |
| 2,067,876    | Campbell       | Jan. 12, 1937  |
| 2,107,390    | Rosmait        | Feb. 8, 1938   |
| 5 2,112,562  | Fisher         | Mar. 29, 1938  |
| 2,125,913    | Goebels        | Aug. 9, 1938   |
| 2,135,261    | Rosmait        | Nov. 1, 1938   |
| 2,186,609    | Kress          | Jan. 9, 1940   |
| 2,200,622    | Hines          | May 14, 1940   |
| 10 2,219,781 | Lowe           | Oct. 29, 1940  |
| 2,288,832    | Pare           | July 7, 1942   |
| 2,330,084    | Scott          | Sept. 21, 1943 |
| 2,375,245    | Pretzel        | May 8, 1945    |
| 2,411,066    | Stevens        | Nov. 12, 1946  |
| 15 2,414,833 | Osborne        | Jan. 28, 1947  |
| 2,492,702    | Neubert et al. | Dec. 27, 1949  |
| 2,563,897    | Wilson         | Aug. 14, 1951  |
| 2,601,671    | Wilson et al.  | June 24, 1952  |

## OTHER REFERENCES

- Collins et al., Paper Trade J., September 25, 1941, pp. 94-99.  
 Price, Paper Trade J., November 20, 1947, pp. 54-59.  
 25 Manufacture of Pulp and Paper 3rd Ed., vol. IV, Sec. 5, pp. 2, 18 and 21 (1938).  
 Sutermeister, Tech. Assoc. Papers, Series XIX, pp. 470 and 473, 1936.